

UNITED STATES PATENT OFFICE.

JAMES R. ROSE, OF EDGEWORTH, PENNSYLVANIA, AND JOHN HARRIS, OF LAKewood, OHIO, ASSIGNEES TO CARBO-OXYGEN COMPANY, OF PITTSBURGH, PENNSYLVANIA, A CORPORATION OF DELAWARE.

GASEOUS FUEL.

1,404,227.

Specification of Letters Patent. Patented Jan. 24, 1922.

No Drawing.

Application filed December 28, 1919. Serial No. 847,454.

To all whom it may concern:

Be it known that we, (1) James R. Rose, (2) John Harris, citizens of the United States, residing at (1) Edgeworth, (2) Lakewood, in the county of (1) Allegheny, (2) Cuyahoga, and State of (1) Pennsylvania, (2) Ohio, have invented a certain new and useful Improvement in Gaseous Fuel, of which the following is a full, clear, 10 and exact description.

This invention relates to gaseous fuel, and particularly to fuels for the cutting and welding of metals wherein a combustible base of hydrogen is employed together with another gas or gases capable of producing within the blow pipe flame a visible or luminous cone whereby the proportions of the combustible gases and oxygen may be conveniently adjusted and the application of the 15 flame to the work is facilitated.

It has been proposed to mix with hydrogen, gases such as illuminating gas and carbon monoxide, the mixture being particularly well suited for certain kinds of work. 20 It is the purpose of this invention to produce a gas, employing hydrogen as such combustible base, which shall be particularly useful for the cutting of alloys, cast steel, corroded, dirty and sluggish iron and 25 steel, as well as cast iron; also for cutting large bodies or masses of metal, as well as for heating such large masses or bodies of metal for the purpose of softening the same. For this purpose we employ a mixture 30 of butane and ethylene with hydrogen in proportions of from 2½% to 12½% by volume each of the butane and ethylene to hydrogen. 35 The mixture is obtained, thereby producing a blow pipe flame the volume and heat units of which will be increased over the volume and heat units produced by the combustion of hydrogen alone with oxygen, to the extent 40 to which the butane and ethylene are present in the mixture. The presence of the butane

and ethylene in the mixture enables the metal to be pre-heated quickly and, in the case of large masses or bodies of such metal, with sufficient rapidity to more than offset 50 the loss of heat through conduction and radiation. This renders the fuel particularly useful for the cutting and heating of such heavy masses of metal, as well as for cutting the special metals of the character 55 set forth hereinbefore.

According to Richards on Metallurgical Calculations, published in 1908, the flame temperature produced by the combustion of the aforesaid gases will exceed 3200° C., and 60 the variations in the percentage of the said gases will cause the following variations in the net B. T. U. per cubic foot of mixture and in the cubic foot of oxygen required for the combustion of a cubic foot of such mixture: 65

No. 1 mixture, 95% H. with 2½% each of the butane and ethylene; net B. T. U.'s 400; cu. ft. of oxygen .718.

No. 2 mixture, 75% H. with 12½% each 70 of butane and ethylene, net B. T. U.'s 925; cu. ft. of oxygen 1.563.

Having thus described our invention, what we claim is:—

1. A gas for cutting, welding and heating 75 purposes consisting of a mixture of butane and ethylene with hydrogen in the proportions of from 2½% to 12½% by volume each of butane and ethylene to hydrogen.

2. A gas for cutting, welding and heating 80 purposes consisting of a mixture of butane and ethylene with hydrogen in proportions not substantially less than 5% by volume of such combined gases to the hydrogen and not materially more than 25% of such combined gases to the hydrogen, the butane and ethylene being present in the proportions of 85 at least 2½% each in such mixture.

In testimony whereof, we hereunto affix our signatures.

JAMES R. ROSE.  
JOHN HARRIS.